



US009018406B2

(12) **United States Patent**  
Forest et al.

(10) Patent No.: US 9,018,406 B2  
(45) Date of Patent: Apr. 28, 2015

- (54) **DICARBOXYLATE-CAPPED ESTOLIDE COMPOUNDS AND METHODS OF MAKING AND USING THE SAME**

(71) Applicants: **Jeremy Forest**, Irvine, CA (US); **Jakob Bredsguard**, Lake Forest, CA (US)

(72) Inventors: **Jeremy Forest**, Irvine, CA (US); **Jakob Bredsguard**, Lake Forest, CA (US)

(73) Assignee: **Biosynthetic Technologies, LLC**, Irvine, CA (US)

(\*) Notice: Subject to any disclaimer, the term of this patent is extended or adjusted under 35 U.S.C. 154(b) by 191 days.

(21) Appl. No.: 13/781,563

(22) Filed: Feb. 28, 2013

(65) **Prior Publication Data**

US 2013/0261325 A1 Oct. 3, 2013

### Related U.S. Application Data

- (60) Provisional application No. 61/616,041, filed on Mar. 27, 2012.

(51) **Int. Cl.**  
*C07C 59/147* (2006.01)  
*C10M 105/42* (2006.01)  
*C10M 105/40* (2006.01)

(52) **U.S. Cl.**  
CPC ..... *C10M 105/42* (2013.01); *C10M 105/40* (2013.01); *C10M 2207/301* (2013.01); *C10N 2230/02* (2013.01); *C10N 2230/10* (2013.01); *C10N 2230/12* (2013.01); *C10N 2230/64* (2013.01)

(58) **Field of Classification Search**

None

See application file for complete search history.

(56) **References Cited**

## U.S. PATENT DOCUMENTS

- |           |     |        |                |         |
|-----------|-----|--------|----------------|---------|
| 2,712,025 | A * | 6/1955 | Rehberg et al. | 549/448 |
| 2,993,860 | A   | 7/1961 | Critchley      |         |
| 4,661,272 | A   | 4/1987 | Marquis et al. |         |
| 5,011,629 | A * | 4/1991 | Billbo         | 554/122 |
| 5,045,586 | A * | 9/1991 | O'Lenick, Jr.  | 524/291 |

|              |    |   |         |                 |       |         |
|--------------|----|---|---------|-----------------|-------|---------|
| 5,219,604    | A  | * | 6/1993  | Kleemann et al. | ..... | 426/531 |
| 5,728,761    | A  | * | 3/1998  | Kuyama et al.   | ..... | 524/306 |
| 8,580,985    | B2 |   | 11/2013 | Thompson et al. |       |         |
| 2009/0264672 | A1 |   | 10/2009 | Abraham et al.  |       |         |

#### OTHER PUBLICATIONS

Pop, L. et al., New complex esters for lubricants, 2007, Revista de Chimie (Bucharest, Romania), 58(8), 805-808, 3 pages abstract.\*  
Meier et al., "Plant oil renewable resources as green alternatives in polymer science", *Chem. Soc. Revs.*, 36: 1788-1802 (2007).

\* cited by examiner

*Primary Examiner* — Yate K Cutliff

(74) *Attorney, Agent, or Firm* — Jeremy Forest

(57) **ABSTRACT**

Described herein are dicarboxylate-capped estolide compound and methods of making the same. Exemplary dicarboxylate-capped estolide compounds include those of the formula



x is, independently for each occurrence, an integer selected from 0 to 20; y is, independently for each occurrence, an integer selected from 0 to 20; W is, independently for each occurrence, selected from  $-\text{CH}_2-$  and  $-\text{CH}=\text{CH}-$ ; z is an integer selected from 1 to 40; n is an integer equal to or greater than 0;  $R_5$  is selected from hydrogen, optionally substituted alkyl that is saturated or unsaturated, and branched or unbranched, and an estolide residue; and  $R_2$  is selected from hydrogen and optionally substituted alkyl that is saturated or unsaturated, and branched or unbranched, wherein each fatty acid chain residue of said at least one compound is independently optionally substituted.

**20 Claims, No Drawings**

1

**DICARBOXYLATE-CAPPED ESTOLIDE COMPOUNDS AND METHODS OF MAKING AND USING THE SAME**

**CROSS-REFERENCE TO RELATED APPLICATIONS**

This application claims the benefit under 35 U.S.C. §119 (e) of U.S. Provisional Patent Application No. 61/616,041, filed Mar. 27, 2012, which is incorporated herein by reference in its entirety for all purposes.

**FIELD**

The present disclosure relates to dicarboxylate-capped estolide compounds. The estolides described herein may be suitable for use as biodegradable base oil stocks and lubricants.

**BACKGROUND**

Lubricant compositions typically comprise a base oil, such as a hydrocarbon base oil, and one or more additives. Estolides present a potential source of biobased, biodegradable oils that may be useful as lubricants and base stocks.

**SUMMARY**

Described herein are estolide compounds, estolide-containing compositions, and methods of making the same. In certain embodiments, such compounds and/or compositions may be useful as base oils and lubricants.

In certain embodiments, the estolide comprises at least one compound of Formula I:



wherein

x is, independently for each occurrence, an integer selected from 0, 1, 2, 3, 4, 5, 6, 7, 8, 9, 10, 11, 12, 13, 14, 15, 16, 17, 18, 19, and 20;

y is, independently for each occurrence, an integer selected from 0, 1, 2, 3, 4, 5, 6, 7, 8, 9, 10, 11, 12, 13, 14, 15, 16, 17, 18, 19, and 20;

z is an integer selected from 1 to 40;

n is an integer equal to or greater than 0;

W is, independently for each occurrence, selected from —CH2— and —CH=CH—;

R5 is selected from hydrogen, optionally substituted alkyl that is saturated or unsaturated, and branched or unbranched, and an estolide residue; and

R2 is selected from hydrogen and optionally substituted alkyl that is saturated or unsaturated, and branched or unbranched,

2

wherein each fatty acid chain residue of said at least one compound is independently optionally substituted.

In certain embodiments, the estolide comprises at least one compound of Formula II:



wherein

n is an integer equal to or greater than 0;

R1 is a saturated or unsaturated and branched or unbranched alkyl substituted with at least one of —CO2H or —C(O)O(alkyl), wherein (alkyl) is optionally substituted;

R2 is selected from hydrogen and optionally substituted alkyl that is saturated or unsaturated, and branched or unbranched; and

R3 and R4, independently for each occurrence, are selected from optionally substituted alkyl that is saturated or unsaturated, and branched or unbranched.

**DETAILED DESCRIPTION**

The use of lubricants and lubricant-containing compositions may result in the dispersion of such fluids, compounds, and/or compositions in the environment. Petroleum base oils used in common lubricant compositions, as well as additives, are typically non-biodegradable and can be toxic. The present disclosure provides for the preparation and use of compositions comprising partially or fully biodegradable base oils, including base oils comprising one or more estolides.

In certain embodiments, the compositions comprising one or more estolides are partially or fully biodegradable and thereby pose diminished risk to the environment. In certain embodiments, the compositions meet guidelines set for by the Organization for Economic Cooperation and Development (OECD) for degradation and accumulation testing. The OECD has indicated that several tests may be used to determine the “ready biodegradability” of organic chemicals.

Aerobic ready biodegradability by OECD 301D measures the mineralization of the test sample to CO2 in closed aerobic microorganisms that simulate an aerobic aquatic environment, with microorganisms seeded from a waste-water treatment plant. OECD 301D is considered representative of most

aerobic environments that are likely to receive waste materials. Aerobic “ultimate biodegradability” can be determined by OECD 302D. Under OECD 302D, microorganisms are pre-acclimated to biodegradation of the test material during a pre-incubation period, then incubated in sealed vessels with

relatively high concentrations of microorganisms and enriched mineral salts medium. OECD 302D ultimately determines whether the test materials are completely biodegradable, albeit under less stringent conditions than “ready biodegradability” assays.

As used in the present specification, the following words, phrases and symbols are generally intended to have the meanings as set forth below, except to the extent that the context in

which they are used indicates otherwise. The following abbreviations and terms have the indicated meanings throughout:

A dash (“-”) that is not between two letters or symbols is used to indicate a point of attachment for a substituent. For example, —C(O)NH<sub>2</sub> is attached through the carbon atom.

“Alkoxy” by itself or as part of another substituent refers to a radical —OR<sup>31</sup> where R<sup>31</sup> is alkyl, cycloalkyl, cycloalkylalkyl, aryl, or arylalkyl, which can be substituted, as defined herein. In some embodiments, alkoxy groups have from 1 to 8 carbon atoms. In some embodiments, alkoxy groups have 1, 2, 3, 4, 5, 6, 7, or 8 carbon atoms. Examples of alkoxy groups include, but are not limited to, methoxy, ethoxy, propoxy, butoxy, cyclohexyloxy, and the like.

“Alkyl” by itself or as part of another substituent refers to a saturated or unsaturated, branched, or straight-chain monovalent hydrocarbon radical derived by the removal of one hydrogen atom from a single carbon atom of a parent alkane, alkene, or alkyne. Examples of alkyl groups include, but are not limited to, methyl; ethyls such as ethanyl, ethenyl, and ethynyl; propyls such as propan-1-yl, propan-2-yl, prop-1-en-1-yl, prop-1-en-2-yl, prop-2-en-1-yl (allyl), prop-1-yn-1-yl, prop-2-yn-1-yl, etc.; butyls such as butan-1-yl, butan-2-yl, 2-methyl-propan-1-yl, 2-methyl-propan-2-yl, but-1-en-1-yl, but-1-en-2-yl, 2-methyl-prop-1-en-1-yl, but-2-en-1-yl, but-2-en-2-yl, buta-1,3-dien-1-yl, buta-1,3-dien-2-yl, but-1-yn-1-yl, but-1-yn-3-yl, but-3-yn-1-yl, etc.; and the like.

Unless otherwise indicated, the term “alkyl” is specifically intended to include groups having any degree or level of saturation, i.e., groups having exclusively single carbon-carbon bonds, groups having one or more double carbon-carbon bonds, groups having one or more triple carbon-carbon bonds, and groups having mixtures of single, double, and triple carbon-carbon bonds. Where a specific level of saturation is intended, the terms “alkanyl,” “alkenyl,” and “alkynyl” are used. In certain embodiments, an alkyl group comprises from 1 to 40 carbon atoms, in certain embodiments, from 1 to 22 or 1 to 18 carbon atoms, in certain embodiments, from 1 to 16 or 1 to 8 carbon atoms, and in certain embodiments from 1 to 6 or 1 to 3 carbon atoms. In certain embodiments, an alkyl group comprises from 8 to 22 carbon atoms, in certain embodiments, from 8 to 18 or 8 to 16. In some embodiments, the alkyl group comprises from 3 to 20 or 7 to 17 carbons. In some embodiments, the alkyl group comprises 1, 2, 3, 4, 5, 6, 7, 8, 9, 10, 11, 12, 13, 14, 15, 16, 17, 18, 19, 20, 21, or 22 carbon atoms.

“Aryl” by itself or as part of another substituent refers to a monovalent aromatic hydrocarbon radical derived by the removal of one hydrogen atom from a single carbon atom of a parent aromatic ring system. Aryl encompasses 5- and 6-membered carbocyclic aromatic rings, for example, benzene; bicyclic ring systems wherein at least one ring is carbocyclic and aromatic, for example, naphthalene, indane, and tetralin; and tricyclic ring systems wherein at least one ring is carbocyclic and aromatic, for example, fluorene. Aryl encompasses multiple ring systems having at least one carbocyclic aromatic ring fused to at least one carbocyclic aromatic ring, cycloalkyl ring, or heterocycloalkyl ring. For example, aryl includes 5- and 6-membered carbocyclic aromatic rings fused to a 5- to 7-membered non-aromatic heterocycloalkyl ring containing one or more heteroatoms chosen from N, O, and S. For such fused, bicyclic ring systems wherein only one of the rings is a carbocyclic aromatic ring, the point of attachment may be at the carbocyclic aromatic ring or the heterocycloalkyl ring. Examples of aryl groups include, but are not limited to, groups derived from aceanthrylene, acenaphthylene, acephenanthrylene, anthracene, azulene, benzene, chry-

sene, coronene, fluoranthene, fluorene, hexacene, hexaphene, hexylene, as-indacene, s-indacene, indane, indene, naphthalene, octacene, octaphene, octalene, ovalene, penta-2,4-diene, pentacene, pentalene, pentaphene, perylene, phenalene, phenanthrene, picene, pleiadene, pyrene, pyranthrene, rubicene, triphenylene, trinaphthalene, and the like. In certain embodiments, an aryl group can comprise from 5 to 20 carbon atoms, and in certain embodiments, from 5 to 12 carbon atoms. In certain embodiments, an aryl group can comprise 5, 6, 7, 8, 9, 10, 11, 12, 13, 14, 15, 16, 17, 18, 19, or 20 carbon atoms. Aryl, however, does not encompass or overlap in any way with heteroaryl, separately defined herein. Hence, a multiple ring system in which one or more carbocyclic aromatic rings is fused to a heterocycloalkyl aromatic ring, is heteroaryl, not aryl, as defined herein.

“Arylalkyl” by itself or as part of another substituent refers to an acyclic alkyl radical in which one of the hydrogen atoms bonded to a carbon atom, typically a terminal or sp<sup>3</sup> carbon atom, is replaced with an aryl group. Examples of arylalkyl groups include, but are not limited to, benzyl, 2-phenylethyl-1-yl, 2-phenylethen-1-yl, naphthylmethyl, 2-naphthylethyl-1-yl, 2-naphthylethen-1-yl, naphthobenzyl, 2-naphthophenylethan-1-yl, and the like. Where specific alkyl moieties are intended, the nomenclature arylalkanyl, arylalkenyl, or arylalkynyl is used. In certain embodiments, an arylalkyl group is C<sub>7-30</sub> arylalkyl, e.g., the alkanyl, alkenyl, or alkynyl moiety of the arylalkyl group is C<sub>1-10</sub> and the aryl moiety is C<sub>6-20</sub>, and in certain embodiments, an arylalkyl group is C<sub>7-20</sub> arylalkyl, e.g., the alkanyl, alkenyl, or alkynyl moiety of the arylalkyl group is C<sub>1-8</sub> and the aryl moiety is C<sub>6-12</sub>.

Estolide “base oil” and “base stock”, unless otherwise indicated, refer to any composition comprising one or more estolide compounds. It should be understood that an estolide “base oil” or “base stock” is not limited to compositions for a particular use, and may generally refer to compositions comprising one or more estolides, including mixtures of estolides. Estolide base oils and base stocks can also include compounds other than estolides.

“Compounds” refers to compounds encompassed by structural Formula I and II herein and includes any specific compounds within the formula whose structure is disclosed herein. Compounds may be identified either by their chemical structure and/or chemical name. When the chemical structure and chemical name conflict, the chemical structure is determinative of the identity of the compound. The compounds described herein may contain one or more chiral centers and/or double bonds and therefore may exist as stereoisomers such as double-bond isomers (i.e., geometric isomers), enantiomers, or diastereomers. Accordingly, any chemical structures within the scope of the specification depicted, in whole or in part, with a relative configuration encompass all possible enantiomers and stereoisomers of the illustrated compounds including the stereoisomerically pure form (e.g., geometrically pure, enantiomerically pure, or diastereomerically pure) and enantiomeric and stereoisomeric mixtures. Enantiomeric and stereoisomeric mixtures may be resolved into their component enantiomers or stereoisomers using separation techniques or chiral synthesis techniques well known to the skilled artisan.

For the purposes of the present disclosure, “chiral compounds” are compounds having at least one center of chirality (i.e. at least one asymmetric atom, in particular at least one asymmetric C atom), having an axis of chirality, a plane of chirality or a screw structure. “Achiral compounds” are compounds which are not chiral.

Compounds of Formula I and II include, but are not limited to, optical isomers of compounds of Formula I and II, race-

mates thereof, and other mixtures thereof. In such embodiments, the single enantiomers or diastereomers, i.e., optically active forms, can be obtained by asymmetric synthesis or by resolution of the racemates. Resolution of the racemates may be accomplished by, for example, chromatography, using, for example a chiral high-pressure liquid chromatography (HPLC) column. However, unless otherwise stated, it should be assumed that Formula I and II cover all asymmetric variants of the compounds described herein, including isomers, racemates, enantiomers, diastereomers, and other mixtures thereof. In addition, compounds of Formula I and II include Z- and E-forms (e.g., cis- and trans-forms) of compounds with double bonds. The compounds of Formula I and II may also exist in several tautomeric forms including the enol form, the keto form, and mixtures thereof. Accordingly, the chemical structures depicted herein encompass all possible tautomeric forms of the illustrated compounds.

“Cycloalkyl” by itself or as part of another substituent refers to a saturated or unsaturated cyclic alkyl radical. Where a specific level of saturation is intended, the nomenclature “cycloalkanyl” or “cycloalkenyl” is used. Examples of cycloalkyl groups include, but are not limited to, groups derived from cyclopropane, cyclobutane, cyclopentane, cyclohexane, and the like. In certain embodiments, a cycloalkyl group is C<sub>3-15</sub> cycloalkyl, and in certain embodiments, C<sub>3-12</sub> cycloalkyl or C<sub>5-12</sub> cycloalkyl. In certain embodiments, a cycloalkyl group is a C<sub>5</sub>, C<sub>6</sub>, C<sub>7</sub>, C<sub>8</sub>, C<sub>9</sub>, C<sub>10</sub>, C<sub>11</sub>, C<sub>12</sub>, C<sub>13</sub>, C<sub>14</sub>, or C<sub>15</sub> cycloalkyl.

“Cycloalkylalkyl” by itself or as part of another substituent refers to an acyclic alkyl radical in which one of the hydrogen atoms bonded to a carbon atom, typically a terminal or sp<sup>3</sup> carbon atom, is replaced with a cycloalkyl group. Where specific alkyl moieties are intended, the nomenclature cycloalkylalkanyl, cycloalkylalkenyl, or cycloalkylalkynyl is used. In certain embodiments, a cycloalkylalkyl group is C<sub>7-30</sub> cycloalkylalkyl, e.g., the alkanyl, alkenyl, or alkynyl moiety of the cycloalkylalkyl group is C<sub>1-10</sub> and the cycloalkyl moiety is C<sub>6-20</sub>, and in certain embodiments, a cycloalkylalkyl group is C<sub>7-20</sub> cycloalkylalkyl, e.g., the alkanyl, alkenyl, or alkynyl moiety of the cycloalkylalkyl group is C<sub>1-8</sub> and the cycloalkyl moiety is C<sub>4-20</sub> or C<sub>6-12</sub>.

“Halogen” refers to a fluoro, chloro, bromo, or iodo group.

“Heteroaryl” by itself or as part of another substituent refers to a monovalent heteroaromatic radical derived by the removal of one hydrogen atom from a single atom of a parent heteroaromatic ring system. Heteroaryl encompasses multiple ring systems having at least one aromatic ring fused to at least one other ring, which can be aromatic or non-aromatic in which at least one ring atom is a heteroatom. Heteroaryl encompasses 5- to 12-membered aromatic, such as 5- to 7-membered, monocyclic rings containing one or more, for example, from 1 to 4, or in certain embodiments, from 1 to 3, heteroatoms chosen from N, O, and S, with the remaining ring atoms being carbon; and bicyclic heterocycloalkyl rings containing one or more, for example, from 1 to 4, or in certain embodiments, from 1 to 3, heteroatoms chosen from N, O, and S, with the remaining ring atoms being carbon and wherein at least one heteroatom is present in an aromatic ring. For example, heteroaryl includes a 5- to 7-membered heterocycloalkyl, aromatic ring fused to a 5- to 7-membered cycloalkyl ring. For such fused, bicyclic heteroaryl ring systems wherein only one of the rings contains one or more heteroatoms, the point of attachment may be at the heteroaromatic ring or the cycloalkyl ring. In certain embodiments, when the total number of N, S, and O atoms in the heteroaryl group exceeds one, the heteroatoms are not adjacent to one another. In certain embodiments, the total number of N, S, and

O atoms in the heteroaryl group is not more than two. In certain embodiments, the total number of N, S, and O atoms in the aromatic heterocycle is not more than one. Heteroaryl does not encompass or overlap with aryl as defined herein.

Examples of heteroaryl groups include, but are not limited to, groups derived from acridine, arsindole, carbazole, β-carboline, chromane, chromene, cinnoline, furan, imidazole, indazole, indole, indoline, indolizine, isobenzofuran, isochromene, isoindole, isoindoline, isoquinoline, isothiazole, isoxazole, naphthyridine, oxadiazole, oxazole, perimidine, phenanthridine, phenanthroline, phenazine, phthalazine, pteridine, purine, pyran, pyrazine, pyrazole, pyridazine, pyridine, pyrimidine, pyrrole, pyrrolizine, quinazoline, quinoline, quinolizine, quinoxaline, tetrazole, thiadiazole, thiazole, thiophene, triazole, xanthene, and the like. In certain embodiments, a heteroaryl group is from 5- to 20-membered heteroaryl, and in certain embodiments from 5- to 12-membered heteroaryl or from 5- to 10-membered heteroaryl. In certain embodiments, a heteroaryl group is a 5-, 6-, 7-, 8-, 9-, 10-, 11-, 12-, 13-, 14-, 15-, 16-, 17-, 18-, 19-, or 20-membered heteroaryl. In certain embodiments heteroaryl groups are those derived from thiophene, pyrrole, benzothiophene, benzofuran, indole, pyridine, quinoline, imidazole, oxazole, and pyrazine.

“Heteroarylalkyl” by itself or as part of another substituent refers to an acyclic alkyl radical in which one of the hydrogen atoms bonded to a carbon atom, typically a terminal or sp<sup>3</sup> carbon atom, is replaced with a heteroaryl group. Where specific alkyl moieties are intended, the nomenclature heteroarylalkanyl, heteroarylalkenyl, or heteroarylalkynyl is used. In certain embodiments, a heteroarylalkyl group is a 6- to 30-membered heteroarylalkyl, e.g., the alkanyl, alkenyl, or alkynyl moiety of the heteroarylalkyl is 1- to 10-membered and the heteroaryl moiety is a 5- to 20-membered heteroaryl, and in certain embodiments, 6- to 20-membered heteroarylalkyl, e.g., the alkanyl, alkenyl, or alkynyl moiety of the heteroarylalkyl is 1- to 8-membered and the heteroaryl moiety is a 5- to 12-membered heteroaryl.

“Heterocycloalkyl” by itself or as part of another substituent refers to a partially saturated or unsaturated cyclic alkyl radical in which one or more carbon atoms (and any associated hydrogen atoms) are independently replaced with the same or different heteroatom. Examples of heteroatoms to replace the carbon atom(s) include, but are not limited to, N, P, O, S, Si, etc. Where a specific level of saturation is intended, the nomenclature “heterocycloalkanyl” or “heterocycloalkenyl” is used. Examples of heterocycloalkyl groups include, but are not limited to, groups derived from epoxides, azirines, thiiranes, imidazolidine, morpholine, piperazine, piperidine, pyrazolidine, pyrrolidine, quinuclidine, and the like.

“Heterocycloalkylalkyl” by itself or as part of another substituent refers to an acyclic alkyl radical in which one of the hydrogen atoms bonded to a carbon atom, typically a terminal or sp<sup>3</sup> carbon atom, is replaced with a heterocycloalkyl group. Where specific alkyl moieties are intended, the nomenclature heterocycloalkylalkanyl, heterocycloalkylalkenyl, or heterocycloalkylalkynyl is used. In certain embodiments, a heterocycloalkylalkyl group is a 6- to 30-membered heterocycloalkylalkyl, e.g., the alkanyl, alkenyl, or alkynyl moiety of the heterocycloalkylalkyl is 1- to 10-membered and the heterocycloalkyl moiety is a 5- to 20-membered heterocycloalkyl, and in certain embodiments, 6- to 20-membered heterocycloalkylalkyl, e.g., the alkanyl, alkenyl, or alkynyl moiety of the heterocycloalkylalkyl is 1- to 8-membered and the heterocycloalkyl moiety is a 5- to 12-membered heterocycloalkyl.

"Mixture" refers to a collection of molecules or chemical substances. Each component in a mixture can be independently varied. A mixture may contain, or consist essentially of, two or more substances intermingled with or without a constant percentage composition, wherein each component may or may not retain its essential original properties, and where molecular phase mixing may or may not occur. In mixtures, the components making up the mixture may or may not remain distinguishable from each other by virtue of their chemical structure.

"Parent aromatic ring system" refers to an unsaturated cyclic or polycyclic ring system having a conjugated  $\pi$  (pi) electron system. Included within the definition of "parent aromatic ring system" are fused ring systems in which one or more of the rings are aromatic and one or more of the rings are saturated or unsaturated, such as, for example, fluorene, indane, indene, phenalene, etc. Examples of parent aromatic ring systems include, but are not limited to, aceanthrylene, acenaphthylene, acephenanthrylene, anthracene, azulene, benzene, chrysene, coronene, fluoranthene, fluorene, hexacene, hexaphene, hexylene, as-indacene, s-indacene, indane, indene, naphthalene, octacene, octaphene, octalene, ovalene, penta-2,4-diene, pentacene, pentalene, pentaphene, perylene, phenalene, phenanthrene, picene, pleiadene, pyrene, pyranthrene, rubicene, triphenylene, trinaphthalene, and the like.

"Parent heteroaromatic ring system" refers to a parent aromatic ring system in which one or more carbon atoms (and any associated hydrogen atoms) are independently replaced with the same or different heteroatom. Examples of heteroatoms to replace the carbon atoms include, but are not limited to, N, P, O, S, Si, etc. Specifically included within the definition of "parent heteroaromatic ring systems" are fused ring systems in which one or more of the rings are aromatic and one or more of the rings are saturated or unsaturated, such as, for example, arsindole, benzodioxan, benzofuran, chromane, chromene, indole, indoline, xanthene, etc. Examples of parent heteroaromatic ring systems include, but are not limited to, arsindole, carbazole,  $\beta$ -carboline, chromane, chromene, cinnoline, furan, imidazole, indazole, indole, indoline, indolizine, isobenzofuran, isochromene, isoindole, isoquinoline, isothiazole, isoxazole, naphthyridine, oxadiazole, oxazole, perimidine, phenanthridine, phenanthroline, phenazine, phthalazine, pteridine, purine, pyran, pyrazine, pyrazole, pyridazine, pyridine, pyrimidine, pyrrole, pyrrolizine, quinazoline, quinoline, quinolizine, quinoxaline, tetrazole, thiadiazole, thiazole, thiophene, triazole, xanthene, and the like.

"Substituted" refers to a group in which one or more hydrogen atoms are independently replaced with the same or different substituent(s). Examples of substituents include, but are not limited to,  $-R^{64}$ ,  $-R^{60}$ ,  $-O^-$ ,  $-OH$ ,  $-O$ ,  $-OR^{60}$ ,  $-SR^{60}$ ,  $-S^-$ ,  $=S$ ,  $-NR^{60}R^{61}$ ,  $=NR^{60}$ ,  $CN$ ,  $-CF_3$ ,  $-OCN$ ,  $-SCN$ ,  $-NO$ ,  $-NO_2$ ,  $=N_2$ ,  $-N_3$ ,  $-S(O)_2O$ ,  $-S(O)_2OH$ ,  $-S(O)_2R^{60}$ ,  $-OS(O)_2O^-$ ,  $-OS(O)_2R^{60}$ ,  $-P(O)(O^-)_2$ ,  $-P(O)(OR^{60})(O^-)$ ,  $-OP(O)(OR^{60})(OR^{61})$ ,  $-C(O)R^{60}$ ,  $-C(S)R^{60}$ ,  $-C(O)OR^{60}$ ,  $-C(O)NR^{60}R^{61}$ ,  $-C(O)O^-$ ,  $-C(S)OR^{60}$ ,  $-NR^{62}C(O)NR^{60}R^{61}$ ,  $NR^{62}C(S)NR^{60}R^{61}$ ,  $-NR^{62}C(NR^{63})NR^{60}R^{61}$ ,  $-C(NR^{62})NR^{60}R^{61}$ ,  $-S(O)_2$ ,  $NR^{60}R^{61}$ ,  $-NR^{63}S(O)_2R^{60}$ ,  $NR^{63}C(O)R^{60}$ , and  $-S(O)R^{60}$ ;

wherein each  $-R^{64}$  is independently a halogen; each  $R^{60}$  and  $R^{61}$  are independently alkyl, substituted alkyl, alkoxy, substituted alkoxy, cycloalkyl, substituted cycloalkyl, heterocycloalkyl, substituted heterocycloalkyl, aryl, substituted aryl, heteroaryl, substituted heteroaryl, arylalkyl, substituted arylalkyl, heteroarylalkyl, or substituted heteroarylalkyl, or

$R^{60}$  and  $R^{61}$  together with the nitrogen atom to which they are bonded form a heterocycloalkyl, substituted heterocycloalkyl, heteroaryl, or substituted heteroaryl ring, and  $R^{62}$  and  $R^{63}$  are independently alkyl, substituted alkyl, aryl, substituted aryl, arylalkyl, substituted arylalkyl, cycloalkyl, substituted cycloalkyl, heterocycloalkyl, substituted heterocycloalkyl, heteroaryl, substituted heteroaryl, heteroarylalkyl, or substituted heteroarylalkyl, or  $R^{62}$  and  $R^{63}$  together with the atom to which they are bonded form one or more heterocycloalkyl, substituted heterocycloalkyl, heteroaryl, or substituted heteroaryl rings;

wherein the "substituted" substituents, as defined above for  $R^{60}$ ,  $R^{61}$ ,  $R^{62}$ , and  $R^{63}$ , are substituted with one or more, such as one, two, or three, groups independently selected from alkyl, -alkyl-OH,  $-O$ -haloalkyl, -alkyl-NH<sub>2</sub>, alkoxy, cycloalkyl, cycloalkylalkyl, heterocycloalkyl, heterocycloalkylalkyl, aryl, heteroaryl, arylalkyl, heteroarylalkyl,  $-O^-$ ,  $-OH$ ,  $=O$ ,  $-O$ -alkyl,  $-O$ -aryl,  $-O$ -heteroarylalkyl,  $-O$ -cycloalkyl,  $-O$ -heterocycloalkyl,  $-SH$ ,  $-S^-$ ,  $=S$ ,  $-S$ -alkyl,  $-S$ -aryl,  $-S$ -heteroarylalkyl,  $-S$ -cycloalkyl,  $-S$ -heterocycloalkyl,  $-NH_2$ ,  $=NH$ ,  $-CN$ ,  $-CF_3$ ,  $-OCN$ ,  $-SCN$ ,  $-NO$ ,  $-NO_2$ ,  $=N_2$ ,  $-N_3$ ,  $-S(O)_2O$ ,  $-S(O)_2$ ,  $-S(O)_2OH$ ,  $-OS(O)_2O$ ,  $-SO_2$  (alkyl),  $-SO_2$ (phenyl),  $-SO_2$ (haloalkyl),  $-SO_2NH_2$ ,  $-SO_2NH$ (alkyl),  $-SO_2NH$ (phenyl),  $-P(O)(O^-)_2$ ,  $-P(O)(O-alkyl)(O-alkyl)$ ,  $-CO_2H$ ,  $-C(O)O$ (alkyl),  $-CON(alkyl)(alkyl)$ ,  $-CONH(alkyl)$ ,  $-CONH_2$ ,  $-C(O)(alkyl)$ ,  $-C(O)(phenyl)$ ,  $-C(O)(haloalkyl)$ ,  $-OC(O)(alkyl)$ ,  $-N(alkyl)(alkyl)$ ,  $-NH(alkyl)$ ,  $-N(alkyl)(alkylphenyl)$ ,  $-NH(alkylphenyl)$ ,  $-NHC(O)(alkyl)$ ,  $-NHC(O)(phenyl)$ ,  $-N(alkyl)C(O)(alkyl)$ , and  $-N(alkyl)C(O)(phenyl)$ .

As used in this specification and the appended claims, the articles "a," "an," and "the" include plural referents unless expressly and unequivocally limited to one referent.

All numerical ranges herein include all numerical values and ranges of all numerical values within the recited range of numerical values.

The present disclosure relates to estolide compounds, compositions and methods of making the same. In certain embodiments, the present disclosure also relates to estolide compounds, compositions comprising estolide compounds, high- and low-viscosity base oil stocks and lubricants, the synthesis of such compounds, and the formulation of such compositions. In certain embodiments, the estolide compounds described herein comprise dicarboxylate-capped estolides, diestolides comprising a dicarboxylate linker, and mixtures thereof.

In certain embodiments estolide compounds are described, wherein the estolides comprise at least one compound of Formula I:



wherein

x is, independently for each occurrence, an integer selected from 0, 1, 2, 3, 4, 5, 6, 7, 8, 9, 10, 11, 12, 13, 14, 15, 16, 17, 18, 19, and 20;

y is, independently for each occurrence, an integer selected from 0, 1, 2, 3, 4, 5, 6, 7, 8, 9, 10, 11, 12, 13, 14, 15, 16, 17, 18, 19, and 20;

z is an integer selected from 1 to 40;

n is an integer equal to or greater than 0;

W is, independently for each occurrence, selected from  $-\text{CH}_2-$  and  $-\text{CH}=\text{CH}-$ ;

$R_5$  is selected from hydrogen, optionally substituted alkyl that is saturated or unsaturated, and branched or unbranched, and an estolide residue; and

$R_2$  is selected from hydrogen and optionally substituted alkyl that is saturated or unsaturated, and branched or unbranched,

wherein each fatty acid chain residue of said at least one compound is independently optionally substituted.

In certain embodiments, the estolide comprises at least one compound of Formula II:



Formula II

wherein

n is an integer equal to or greater than 0;

$R_1$  is a saturated or unsaturated and branched or unbranched alkyl substituted with at least one of  $-\text{CO}_2\text{H}$  or  $-\text{C}(\text{O})\text{O}(\text{alkyl})$ , wherein (alkyl) is optionally substituted;

$R_2$  is selected from hydrogen and optionally substituted alkyl that is saturated or unsaturated, and branched or unbranched; and

$R_3$  and  $R_4$ , independently for each occurrence, are selected from optionally substituted alkyl that is saturated or unsaturated, and branched or unbranched.

In certain embodiments, the composition comprises at least one compound of Formula I, wherein  $R_5$  and/or  $R_2$  are hydrogen.

The terms "chain" or "fatty acid chain" or "fatty acid chain residue," as used with respect to the estolide compounds of Formula I and II, refer to one or more of the fatty acid residues incorporated in estolide compounds, e.g.,  $R_3$  or  $R_4$  of Formula II, or the structures represented by  $\text{CH}_3(\text{CH}_2)_n\text{CH}(\text{CH}_2)-\text{C}(\text{O})\text{O}-$  or  $R_5\text{OC}(\text{O})(\text{CH}_2)_z\text{C}(\text{O})\text{O}-$  in Formula I.

The residue represented at the top of each of Formula I and II is an example of what may be referred to as a "cap" or "capping material," as it "caps" the top of the estolide (e.g.,  $R_1$  of Formula II). The capping group may be an organic diacid residue of general formula  $\text{HOC}(\text{O})\text{-alkyl-C}(\text{O})\text{O}-$ , i.e., a dicarboxylic acid comprising a substituted or unsubstituted, saturated or unsaturated, and/or branched or unbranched alkyl residue as defined herein. In certain embodiments, the "cap" or "capping group" comprises a free carboxylic acid residue, or an esterified carboxylate residue. In certain embodiments, the capping group, regardless of size, is sub-

stituted or unsubstituted, saturated or unsaturated, and/or branched or unbranched. Depending on the manner in which the estolide is synthesized, the terminal carboxylic acid residue of the dicarboxylate cap may remain in its free-acid form after the initial synthesis of the estolide. However, in certain embodiments, in an effort to alter or improve the properties of the estolide, the free carboxylic acid residue of the cap may be reacted with any number of substituents. For example, it may be desirable to react the free acid residue of the dicarboxylate cap with a group selected from alcohols, glycols, amines, or other suitable reactants to provide the corresponding ester, amide, or other reaction products. The cap or capping material may also be referred to as the primary or alpha ( $\alpha$ ) chain.

Depending on the manner in which the estolide is synthesized, in certain embodiments, the cap may comprise the only alkyl residue in the resulting estolide that is unsaturated. In certain embodiments, it may be desirable to use a saturated dicarboxylic acid cap to increase the overall saturation of the estolide and/or to increase the resulting estolide's stability.

For example, in certain embodiments, it may be desirable to provide a method of providing a saturated capped estolide by hydrogenating an unsaturated cap using any suitable methods available to those of ordinary skill in the art. Hydrogenation may be used with various sources of the fatty-acid feedstock, which may include mono- and/or polyunsaturated fatty acids. Without being bound to any particular theory, in certain embodiments, hydrogenating the estolide may help to improve the overall stability of the molecule. However, a fully-hydrogenated estolide, such as an estolide with a larger dicarboxylic acid cap, may exhibit increased pour point temperatures. In certain embodiments, it may be desirable to offset any loss in desirable pour-point characteristics by using shorter, saturated capping materials.

The  $\text{R}_4\text{C}(\text{O})\text{O}-$  of Formula II or structure  $\text{CH}_3(\text{CH}_2)_n\text{CH}$

$(\text{CH}_2)-\text{C}(\text{O})\text{O}-$  of Formula I serve as the "base" or "base chain residue" of the estolide. Depending on the manner in which the estolide is synthesized, the base organic acid or fatty acid residue (in addition to the dicarboxylic acid cap) may be the only residue that remains in its free-acid form after the initial synthesis of the estolide. However, in certain embodiments, in an effort to alter or improve the properties of the estolide, the free acid may be reacted with any number of substituents. For example, it may be desirable to react the free acid estolide with a group selected from alcohols, glycols, amines, or other suitable reactants to provide the corresponding ester, amide, or other reaction products. The base or base chain residue may also be referred to as tertiary or gamma ( $\gamma$ ) chains.

The  $\text{R}_3\text{C}(\text{O})\text{O}-$  of Formula II or structure  $\text{CH}_3(\text{CH}_2)_n\text{CH}$

$(\text{CH}_2)-\text{C}(\text{O})\text{O}-$  of Formula I are linking residues that link the capping material and the base fatty-acid residue together. There may be any number of linking residues in the estolide, including when  $n=0$  and the estolide is in its dimer form. Depending on the manner in which the estolide is prepared, a linking residue may be a fatty acid and may initially be in an unsaturated form during synthesis. In some embodiments, the estolide will be formed when a catalyst is used to produce a carbocation at the fatty acid's site of unsaturation, which is followed by nucleophilic attack on the carbocation by the carboxylic group of another fatty acid. In some embodiments, it may be desirable to have a linking fatty acid that is monounsaturated so that when the fatty acids link together, all of the sites of unsaturation are eliminated. The linking residue(s) may also be referred to as secondary or beta ( $\beta$ ) chains.

As noted above, in certain embodiments, suitable unsaturated fatty acids for preparing the estolides may include any mono- or polyunsaturated fatty acid. For example, monoun-

## 11

saturated fatty acids, along with a suitable catalyst, will form a single carbocation that allows for the addition of a second fatty acid, whereby a single link between two fatty acids is formed. Suitable monounsaturated fatty acids may include, but are not limited to, palmitoleic acid (16:1), vaccenic acid (18:1), oleic acid (18:1), eicosenoic acid (20:1), erucic acid (22:1), and nervonic acid (24:1). In addition, in certain embodiments, polyunsaturated fatty acids may be used to create estolides. Suitable polyunsaturated fatty acids may include, but are not limited to, hexadecatrienoic acid (16:3), alpha-linolenic acid (18:3), stearidonic acid (18:4), eicosatrienoic acid (20:3), eicosatetraenoic acid (20:4), eicosapentaenoic acid (20:5), heneicosapentaenoic acid (21:5), docosapentaenoic acid (22:5), docosahexaenoic acid (22:6), tetracosapentaenoic acid (24:5), tetracosahexaenoic acid (24:6), linoleic acid (18:2), gamma-linoleic acid (18:3), eicosadienoic acid (20:2), dihomo-gamma-linolenic acid (20:3), arachidonic acid (20:4), docosadienoic acid (20:2), adrenic acid (22:4), docosapentaenoic acid (22:5), tetracosatetraenoic acid (22:4), tetracosapentaenoic acid (24:5), pinolenic acid (18:3), podocarpic acid (20:3), rumenic acid (18:2), alpha-calendic acid (18:3), beta-calendic acid (18:3), jacaric acid (18:3), alpha-eleostearic acid (18:3), beta-eleostearic (18:3), catalpic acid (18:3), punicic acid (18:3), rumelenic acid (18:3), alpha-parinaric acid (18:4), beta-parinaric acid (18:4), and boscopeptaenoic acid (20:5). In certain embodiments, hydroxy fatty acids may be polymerized or homopolymerized by reacting the carboxylic acid functionality of one fatty acid with the hydroxy functionality of a second fatty acid. Exemplary hydroxyl fatty acids include, but are not limited to, ricinoleic acid, 6-hydroxystearic acid, 9,10-dihydroxystearic acid, 12-hydroxystearic acid, and 14-hydroxystearic acid. For example, the dicarboxylate-capped estolides described herein may be prepared by condensing one or more hydroxy fatty acids with a dicarboxylic acid.

The process for preparing the estolide compounds described herein may include the use of any natural or synthetic fatty acid source. However, it may be desirable to source the fatty acids from a renewable biological feedstock. Suitable starting materials of biological origin may include plant fats, plant oils, plant waxes, animal fats, animal oils, animal waxes, fish fats, fish oils, fish waxes, algal oils and mixtures thereof. Other potential fatty acid sources may include waste and recycled food-grade fats and oils, fats, oils, and waxes obtained by genetic engineering, fossil fuel-based materials and other sources of the materials desired.

In some embodiments, the compound comprises fatty-acid chains of varying lengths. In some embodiments, x is, independently for each occurrence, an integer selected from 0 to 20, 0 to 18, 0 to 16, 0 to 14, 1 to 12, 1 to 10, 2 to 8, 6 to 8, or 4 to 6. In some embodiments, x is, independently for each occurrence, an integer selected from 7 and 8. In some embodiments, x is, independently for each occurrence, an integer selected from 0, 1, 2, 3, 4, 5, 6, 7, 8, 9, 10, 11, 12, 13, 14, 15, 16, 17, 18, 19, and 20. In certain embodiments, for at least one fatty acid chain residue, x is an integer selected from 7 and 8.

In some embodiments, y is, independently for each occurrence, an integer selected from 0 to 20, 0 to 18, 0 to 16, 0 to 14, 1 to 12, 1 to 10, 2 to 8, 6 to 8, or 4 to 6. In some embodiments, y is, independently for each occurrence, an integer selected from 7 and 8. In some embodiments, y is, independently for each occurrence, an integer selected from 0, 1, 2, 3, 4, 5, 6, 7, 8, 9, 10, 11, 12, 13, 14, 15, 16, 17, 18, 19, and 20. In certain embodiments, for at least one fatty acid chain residue, y is an integer selected from 7 and 8. In some embodiments, for at least one fatty acid chain residue, y is an integer selected from

## 12

0 to 6, or 1 and 2. In certain embodiments, y is, independently for each occurrence, an integer selected from 1 to 6, or 1 and 2.

In some embodiments, x+y is, independently for each chain, an integer selected from 0 to 40, 0 to 20, 10 to 20, or 12 to 18. In some embodiments, x+y is, independently for each chain, an integer selected from 13 to 15. In some embodiments, x+y is 15. In some embodiments, x+y is, independently for each chain, an integer selected from 6, 7, 8, 9, 10, 11, 12, 13, 14, 15, 16, 17, 18, 19, 20, 21, 22, 23, and 24.

In some embodiments, the estolide compound of Formula I or II may comprise any number of fatty acid residues to form an "n-mer" estolide. For example, the estolide may be in its dimer (n=0), trimer (n=1), tetramer (n=2), pentamer (n=3), hexamer (n=4), heptamer (n=5), octamer (n=6), nonamer (n=7), or decamer (n=8) form. In some embodiments, n is an integer selected from 0 to 20, 0 to 18, 0 to 16, 0 to 14, 0 to 12, 0 to 10, 0 to 8, or 0 to 6. In some embodiments, n is an integer selected from 0 to 4. In certain embodiments, n is 0 or greater than 0. In some embodiments, n is 1, wherein said at least one compound of Formula I or II comprises the trimer. In some embodiments, n is greater than 1. In some embodiments, n is an integer selected from 0, 1, 2, 3, 4, 5, 6, 7, 8, 9, 10, 11, 12, 13, 14, 15, 16, 17, 18, 19, and 20.

In certain embodiments, R<sub>5</sub> is selected from hydrogen, optionally substituted alkyl that is saturated or unsaturated, and branched or unbranched, and an estolide residue. In some embodiments, the optionally substituted alkyl group is a C<sub>1</sub> to C<sub>40</sub> alkyl, C<sub>1</sub> to C<sub>22</sub> alkyl or C<sub>1</sub> to C<sub>18</sub> alkyl. In some embodiments, the optionally substituted alkyl group is selected from C<sub>7</sub> to C<sub>17</sub> alkyl. In some embodiments, R<sub>5</sub> is selected from C<sub>7</sub> alkyl, C<sub>9</sub> alkyl, C<sub>11</sub> alkyl, C<sub>13</sub> alkyl, C<sub>15</sub> alkyl, and C<sub>17</sub> alkyl. In some embodiments, R<sub>5</sub> is selected from C<sub>13</sub> to C<sub>17</sub> alkyl, such as from C<sub>13</sub> alkyl, C<sub>15</sub> alkyl, and C<sub>17</sub> alkyl. In some embodiments, R<sub>5</sub> is a C<sub>1</sub>, C<sub>2</sub>, C<sub>3</sub>, C<sub>4</sub>, C<sub>5</sub>, C<sub>6</sub>, C<sub>7</sub>, C<sub>8</sub>, C<sub>9</sub>, C<sub>10</sub>, C<sub>11</sub>, C<sub>12</sub>, C<sub>13</sub>, C<sub>14</sub>, C<sub>15</sub>, C<sub>16</sub>, C<sub>17</sub>, C<sub>18</sub>, C<sub>19</sub>, C<sub>20</sub>, C<sub>21</sub>, or C<sub>22</sub> alkyl.

Depending on the manner in which the estolide is prepared, in certain embodiments, R<sub>5</sub> may be an estolide residue. In certain embodiments, wherein R<sub>5</sub> is an estolide residue, the compound of Formula I may be referred to as a "diestolide." In certain embodiments, the dicarboxylate cap serves as a link between two different fatty acids or fatty acid oligomers. In certain embodiments, R<sub>5</sub> is an estolide residue, wherein the estolide residue comprises the structure of Formula III:



wherein

x', independently for each occurrence, is an integer selected from 0, 1, 2, 3, 4, 5, 6, 7, 8, 9, 10, 11, 12, 13, 14, 15, 16, 17, 18, 19, and 20;

y', independently for each occurrence, is an integer selected from 0, 1, 2, 3, 4, 5, 6, 7, 8, 9, 10, 11, 12, 13, 14, 15, 16, 17, 18, 19, and 20;

n' is an integer equal to or greater than 0; and

$R_6$  is selected from hydrogen and optionally substituted alkyl that is saturated or unsaturated, and branched or unbranched.

In certain embodiments,  $x'$  is, independently for each occurrence, selected from one of the values set forth herein with respect to  $x$ . In certain embodiments,  $y'$  is, independently for each occurrence, selected from one of the values set forth herein with respect to  $y$ . In certain embodiments,  $n'$  is an integer selected from one of the values set forth herein with respect to  $n$ . In certain embodiments,  $R_6$  is selected from one of the groups set forth herein with respect to  $R_2$ .

In certain embodiments,  $z$  is an integer selected from 0 to 40 or 1 to 40. In certain embodiments,  $z$  is an integer greater than 0. In certain embodiments,  $z$  is an integer selected from 1 to 36, 1 to 30, or 1 to 26. In certain embodiments,  $z$  is selected from 1 to 22, 4 to 18, 6 to 16, or 8 to 12. In certain embodiments,  $z$  is 10. In certain embodiments,  $z$  is an integer selected from 0, 1, 2, 3, 4, 5, 6, 7, 8, 9, 10, 11, 12, 13, 14, 15, 16, 17, 18, 19, 20, 21, 22, 23, 24, 25, 26, 27, 28, 29, 30, 31, 32, 33, 34, 35, 36, 37, 38, 39, or 40.

In some embodiments,  $R_1$  is a saturated or unsaturated and branched or unbranched alkyl substituted with at least one of  $—CO_2H$  or  $—C(O)O(alkyl)$ , wherein (alkyl) is optionally substituted. In some embodiments, the alkyl group is a  $C_1$  to  $C_{40}$  alkyl,  $C_1$  to  $C_{22}$  alkyl or  $C_1$  to  $C_{18}$  alkyl. In some embodiments, the alkyl group is selected from  $C_7$  to  $C_{17}$  alkyl. In some embodiments,  $R_1$  is selected from  $C_7$  alkyl,  $C_9$  alkyl,  $C_{11}$  alkyl,  $C_{13}$  alkyl,  $C_{15}$  alkyl, and  $C_{17}$  alkyl. In some embodiments,  $R_1$  is selected from  $C_{13}$  to  $C_{17}$  alkyl, such as from  $C_{13}$  alkyl,  $C_{15}$  alkyl, and  $C_{17}$  alkyl. In some embodiments,  $R_1$  is a  $C_1$ ,  $C_2$ ,  $C_3$ ,  $C_4$ ,  $C_5$ ,  $C_6$ ,  $C_7$ ,  $C_8$ ,  $C_9$ ,  $C_{10}$ ,  $C_{11}$ ,  $C_{12}$ ,  $C_{13}$ ,  $C_{14}$ ,  $C_{15}$ ,  $C_{16}$ ,  $C_{17}$ ,  $C_{18}$ ,  $C_{19}$ ,  $C_{20}$ ,  $C_{21}$ , or  $C_{22}$  alkyl.

In some embodiments,  $R_2$  of Formula I or II is hydrogen or optionally substituted alkyl that is saturated or unsaturated, and branched or unbranched. In some embodiments, the alkyl group is a  $C_1$  to  $C_{40}$  alkyl,  $C_1$  to  $C_{22}$  alkyl or  $C_1$  to  $C_{18}$  alkyl. In some embodiments, the alkyl group is selected from  $C_7$  to  $C_{17}$  alkyl. In some embodiments,  $R_2$  is selected from  $C_7$  alkyl,  $C_9$  alkyl,  $C_{11}$  alkyl,  $C_{13}$  alkyl,  $C_{15}$  alkyl,  $C_{17}$  alkyl, and  $C_{19}$  alkyl. In some embodiments,  $R_2$  is selected from  $C_{13}$  to  $C_{17}$  alkyl, such as from  $C_{13}$  alkyl,  $C_{15}$  alkyl, and  $C_{17}$  alkyl. In some embodiments,  $R_2$  is a  $C_1$ ,  $C_2$ ,  $C_3$ ,  $C_4$ ,  $C_5$ ,  $C_6$ ,  $C_7$ ,  $C_8$ ,  $C_9$ ,  $C_{10}$ ,  $C_{11}$ ,  $C_{12}$ ,  $C_{13}$ ,  $C_{14}$ ,  $C_{15}$ ,  $C_{16}$ ,  $C_{17}$ ,  $C_{18}$ ,  $C_{19}$ ,  $C_{20}$ ,  $C_{21}$ , or  $C_{22}$  alkyl.

In some embodiments,  $R_3$  is an optionally substituted alkyl that is saturated or unsaturated, and branched or unbranched. In some embodiments, the alkyl group is a  $C_1$  to  $C_{40}$  alkyl,  $C_1$  to  $C_{22}$  alkyl or  $C_1$  to  $C_{18}$  alkyl. In some embodiments, the alkyl group is selected from  $C_7$  to  $C_{17}$  alkyl. In some embodiments,  $R_3$  is selected from  $C_7$  alkyl,  $C_9$  alkyl,  $C_{11}$  alkyl,  $C_{13}$  alkyl,  $C_{15}$  alkyl, and  $C_{17}$  alkyl. In some embodiments,  $R_3$  is selected from  $C_{13}$  to  $C_{17}$  alkyl, such as from  $C_{13}$  alkyl,  $C_{15}$  alkyl, and  $C_{17}$  alkyl. In some embodiments,  $R_3$  is a  $C_1$ ,  $C_2$ ,  $C_3$ ,  $C_4$ ,  $C_5$ ,  $C_6$ ,  $C_7$ ,  $C_8$ ,  $C_9$ ,  $C_{10}$ ,  $C_{11}$ ,  $C_{12}$ ,  $C_{13}$ ,  $C_{14}$ ,  $C_{15}$ ,  $C_{16}$ ,  $C_{17}$ ,  $C_{18}$ ,  $C_{19}$ ,  $C_{20}$ ,  $C_{21}$ , or  $C_{22}$  alkyl.

In some embodiments,  $R_4$  is an optionally substituted alkyl that is saturated or unsaturated, and branched or unbranched. In some embodiments, the alkyl group is a  $C_1$  to  $C_{40}$  alkyl,  $C_1$  to  $C_{22}$  alkyl or  $C_1$  to  $C_{18}$  alkyl. In some embodiments, the alkyl group is selected from  $C_7$  to  $C_{17}$  alkyl. In some embodiments,  $R_4$  is selected from  $C_7$  alkyl,  $C_9$  alkyl,  $C_{11}$  alkyl,  $C_{13}$  alkyl,  $C_{15}$  alkyl, and  $C_{17}$  alkyl. In some embodiments,  $R_4$  is selected from  $C_{13}$  to  $C_{17}$  alkyl, such as from  $C_{13}$  alkyl,  $C_{15}$  alkyl, and  $C_{17}$  alkyl. In some embodiments,  $R_4$  is a  $C_1$ ,  $C_2$ ,  $C_3$ ,  $C_4$ ,  $C_5$ ,  $C_6$ ,  $C_7$ ,  $C_8$ ,  $C_9$ ,  $C_{10}$ ,  $C_{11}$ ,  $C_{12}$ ,  $C_{13}$ ,  $C_{14}$ ,  $C_{15}$ ,  $C_{16}$ ,  $C_{17}$ ,  $C_{18}$ ,  $C_{19}$ ,  $C_{20}$ ,  $C_{21}$ , or  $C_{22}$  alkyl.

As noted above, in certain embodiments, it may be possible to manipulate one or more of the estolides' properties by

altering the length of  $R_1$  and/or its degree of saturation. However, in certain embodiments, the level of substitution on  $R_1$  may also be altered to change or even improve the estolides' properties. Without being bound to any particular theory, in certain embodiments, it is believed that the presence of polar substituents on  $R_1$ , such as one or more hydroxy groups, may increase the viscosity of the estolide, while increasing pour point. Accordingly, in some embodiments,  $R_1$  will be unsubstituted or optionally substituted with a group that is not hydroxyl.

In some embodiments, the estolide is in its free-acid form, wherein  $R_2$  and/or  $R_5$  of Formula I are hydrogen, and  $R_2$  is hydrogen and/or  $R_1$  is substituted with  $—CO_2H$  for compounds of Formula II. In some embodiments,  $R_2$  and/or  $R_5$  are independently selected from optionally substituted alkyl that is saturated or unsaturated, and branched or unbranched. In certain embodiments, the  $R_2$  and/or  $R_5$  residue may be independently selected from any desired alkyl group, such as those derived from esterification of the estolide with the alcohols identified in the examples herein. In some embodiments, the alkyl group is selected from  $C_1$  to  $C_{40}$ ,  $C_1$  to  $C_{22}$ ,  $C_3$  to  $C_{20}$ ,  $C_1$  to  $C_{18}$ , or  $C_6$  to  $C_{12}$  alkyl. In some embodiments, the alkyl groups may be selected from  $C_3$  alkyl,  $C_4$  alkyl,  $C_8$  alkyl,  $C_{12}$  alkyl,  $C_{16}$  alkyl,  $C_{18}$  alkyl, and  $C_{20}$  alkyl. For example, in certain embodiments, the alkyl groups may be branched, such as isopropyl, isobutyl, or 2-ethylhexyl. In some embodiments, the alkyl groups may be selected from larger alkyl groups, branched or unbranched, comprising  $C_{12}$  alkyl,  $C_{16}$  alkyl,  $C_{18}$  alkyl, or  $C_{20}$  alkyl. Such groups at the  $R_2$  and/or  $R_5$  position may be derived from esterification of the free-acid estolide using the Jarcol<sup>TM</sup> line of alcohols marketed by Jarchem Industries, Inc. of Newark, N.J., including Jarcol<sup>TM</sup> I-18CG, I-20, I-12, I-16, I-18T, and 85BJ. In certain embodiments,  $R_2$  and/or  $R_5$  may be sourced from certain alcohols to provide branched alkyls such as isostearyl and isopalmityl. It should be understood that such isopalmityl and isostearyl alkyl groups may cover any branched variation of  $C_{16}$  and  $C_{18}$ , respectively. For example, the estolides described herein may comprise highly-branched isopalmityl or isostearyl groups at the  $R_2$  and/or  $R_5$  position, derived from the Fineoxocol<sup>®</sup> line of isopalmityl and isostearyl alcohols marketed by 35 Nissan Chemical America Corporation of Houston, Tex., including Fineoxocol<sup>®</sup> 180, 180N, and 1600. Without being bound to any particular theory, in embodiments, large, highly-branched alkyl groups (e.g., isopalmityl and isostearyl) at the  $R_2$  and/or  $R_5$  position of the estolides can provide at least one way to increase the lubricant's viscosity, while substantially retaining or even reducing its pour point.

In some embodiments, the compounds described herein may comprise a mixture of two or more estolide compounds of Formula I and II. It is possible to characterize the chemical makeup of an estolide, a mixture of estolides, or a composition comprising estolides, by using the compound's, mixture's, or composition's measured estolide number (EN) of compound or composition. The EN represents the average number of fatty acids added to the base fatty acid. The EN also represents the average number of estolide linkages per molecule:

$$EN = n + 1$$

wherein  $n$  is the number of secondary ( $\beta$ ) fatty acids. Accordingly, a single estolide compound will have an EN that is a whole number, for example for dimers, trimers, and tetramers:

$$\text{dimer EN} = 1$$

$$\text{trimer EN} = 2$$

$$\text{tetramer EN} = 3$$

However, a composition comprising two or more estolide compounds may have an EN that is a whole number or a fraction of a whole number. For example, a composition having a 1:1 molar ratio of dimer and trimer would have an EN of 1.5, while a composition having a 1:1 molar ratio of tetramer and trimer would have an EN of 2.5.

In some embodiments, the compositions may comprise a mixture of two or more estolides having an EN that is an integer or fraction of an integer that is greater than 4.5, or even 5.0. In some embodiments, the EN may be an integer or fraction of an integer selected from about 1.0 to about 5.0. In some embodiments, the EN is an integer or fraction of an integer selected from 1.2 to about 4.5. In some embodiments, the EN is selected from a value greater than 1.0, 1.2, 1.4, 1.6, 1.8, 2.0, 2.2, 2.4, 2.6, 2.8, 3.0, 3.2, 3.4, 3.6, 3.8, 4.0, 4.2, 4.4, 4.6, 4.8, 5.0, 5.2, 5.4, 5.6 and 5.8. In some embodiments, the EN is selected from a value less than 1.2, 1.4, 1.6, 1.8, 2.0, 2.2, 2.4, 2.6, 2.8, 3.0, 3.2, 3.4, 3.6, 3.8, 4.0, 4.2, 4.4, 4.6, 4.8, and 5.0, 5.2, 5.4, 5.6, 5.8, and 6.0. In some embodiments, the EN is selected from 1, 1.2, 1.4, 1.6, 1.8, 2.0, 2.2, 2.4, 2.6, 2.8, 3.0, 3.2, 3.4, 3.6, 3.8, 4.0, 4.2, 4.4, 4.6, 4.8, and 5.0, 5.2, 5.4, 5.6, 5.8, and 6.0.

As noted above, it should be understood that the chains of the estolide compounds may be independently optionally substituted, wherein one or more hydrogens are removed and replaced with one or more of the substituents identified herein. Similarly, two or more of the hydrogen residues may be removed to provide one or more sites of unsaturation, such as a cis or trans double bond. Further, the chains may optionally comprise branched hydrocarbon residues. For example, in some embodiments the estolides described herein may comprise at least one compound of Formula II:



Formula II

wherein

n is an integer equal to or greater than 0;

R<sub>1</sub> is a saturated or unsaturated and branched or unbranched alkyl substituted with at least one of —CO<sub>2</sub>H or —C(O)O(alkyl), wherein (alkyl) is optionally substituted;

R<sub>2</sub> is selected from hydrogen and optionally substituted alkyl that is saturated or unsaturated, and branched or unbranched; and

R<sub>3</sub> and R<sub>4</sub>, independently for each occurrence, are selected from optionally substituted alkyl that is saturated or unsaturated, and branched or unbranched.

In certain embodiments, n is 0 or greater than 0. In some embodiments, n is an integer selected from 1 to 20. In some embodiments, n is an integer selected from 1 to 12. In some embodiments, n is an integer selected from 0, 1, 2, 3, 4, 5, 6, 7, 8, 9, 10, 11, 12, 13, 14, 15, 16, 17, 18, 19 and 20. In some embodiments, one or more R<sub>3</sub> differs from one or more other R<sub>3</sub> in a compound of Formula II. In some embodiments, one or more R<sub>3</sub> differs from R<sub>4</sub> in a compound of Formula II. In some embodiments, if the compounds of Formula II are pre-

pared from one or more polyunsaturated fatty acids, it is possible that one or more of R<sub>3</sub> and R<sub>4</sub> will have one or more sites of unsaturation. In some embodiments, if the compounds of Formula II are prepared from one or more branched fatty acids, it is possible that one or more of R<sub>3</sub> and R<sub>4</sub> will be branched.

In some embodiments, R<sub>3</sub> and R<sub>4</sub> can be CH<sub>3</sub>(CH<sub>2</sub>)<sub>x</sub>CH(CH<sub>2</sub>)<sub>y</sub>—, where x is, independently for each occurrence, an integer selected from 0, 1, 2, 3, 4, 5, 6, 7, 8, 9, 10, 11, 12, 13, 14, 15, 16, 17, 18, 19, and 20, and y is, independently for each occurrence, an integer selected from 0, 1, 2, 3, 4, 5, 6, 7, 8, 9, 10, 11, 12, 13, 14, 15, 16, 17, 18, 19, and 20. Where both R<sub>3</sub> and R<sub>4</sub> are CH<sub>3</sub>(CH<sub>2</sub>)<sub>x</sub>CH(CH<sub>2</sub>)<sub>y</sub>—, the compounds may be compounds according to Formula I.

Without being bound to any particular theory, in certain embodiments, altering the EN produces estolides having desired viscometric properties while substantially retaining or even reducing pour point. For example, in some embodiments the estolides exhibit a decreased pour point upon increasing the EN value. Accordingly, in certain embodiments, a method is provided for retaining or decreasing the pour point of an estolide base oil by increasing the EN of the base oil, or a method is provided for retaining or decreasing the pour point of a composition comprising an estolide base oil by increasing the EN of the base oil. In some embodiments, the method comprises: selecting an estolide base oil having an initial EN and an initial pour point; and removing at least a portion of the base oil, said portion exhibiting an EN that is less than the initial EN of the base oil, wherein the resulting estolide base oil exhibits an EN that is greater than the initial EN of the base oil, and a pour point that is equal to or lower than the initial pour point of the base oil. In some embodiments, the selected estolide base oil is prepared by oligomerizing at least one first unsaturated fatty acid with at least one second unsaturated fatty acid and/or saturated fatty acid. In some embodiments, the removing at least a portion of the base oil is accomplished by distillation, chromatography, membrane separation, phase separation, affinity separation, solvent extraction, or combinations thereof. In some embodiments, the distillation takes place at a temperature and/or pressure that is suitable to separate the estolide base oil into different “cuts” that individually exhibit different EN values. In some embodiments, this may be accomplished by subjecting the base oil temperature of at least about 250° C. and an absolute pressure of no greater than about 25 microns. In some embodiments, the distillation takes place at a temperature range of about 250° C. to about 310° C. and an absolute pressure range of about 10 microns to about 25 microns.

In some embodiments, estolide compounds and compositions exhibit an EN that is greater than or equal to 1, such as an integer or fraction of an integer selected from about 1.0 to about 2.0. In some embodiments, the EN is an integer or fraction of an integer selected from about 1.0 to about 1.6. In some embodiments, the EN is a fraction of an integer selected from about 1.1 to about 1.5. In some embodiments, the EN is selected from a value greater than 1.0, 1.1, 1.2, 1.3, 1.4, 1.5, 1.6, 1.7, 1.8, and 1.9. In some embodiments, the EN is selected from a value less than 1.1, 1.2, 1.3, 1.4, 1.5, 1.6, 1.7, 1.8, 1.9, and 2.0.

In some embodiments, the EN is greater than or equal to 1.5, such as an integer or fraction of an integer selected from about 1.8 to about 2.8. In some embodiments, the EN is an integer or fraction of an integer selected from about 2.0 to about 2.6. In some embodiments, the EN is a fraction of an integer selected from about 2.1 to about 2.5. In some embodiments, the EN is selected from a value greater than 1.8, 1.9, 2.0, 2.1, 2.2, 2.3, 2.4, 2.5, 2.6, and 2.7. In some embodiments,

the EN is selected from a value less than 1.9, 2.0, 2.1, 2.2, 2.3, 2.4, 2.5, 2.6, 2.7, and 2.8. In some embodiments, the EN is about 1.8, 2.0, 2.2, 2.4, 2.6, or 2.8.

In some embodiments, the EN is greater than or equal to about 4, such as an integer or fraction of an integer selected from about 4.0 to about 5.0. In some embodiments, the EN is a fraction of an integer selected from about 4.2 to about 4.8. In some embodiments, the EN is a fraction of an integer selected from about 4.3 to about 4.7. In some embodiments, the EN is selected from a value greater than 4.0, 4.1, 4.2, 4.3, 4.4, 4.5, 4.6, 4.7, 4.8, and 4.9. In some embodiments, the EN is selected from a value less than 4.1, 4.2, 4.3, 4.4, 4.5, 4.6, 4.7, 4.8, 4.9, and 5.0. In some embodiments, the EN is about 4.0, 4.2, 4.4, 4.6, 4.8, or 5.0.

In some embodiments, the EN is greater than or equal to about 5, such as an integer or fraction of an integer selected from about 5.0 to about 6.0. In some embodiments, the EN is a fraction of an integer selected from about 5.2 to about 5.8. In some embodiments, the EN is a fraction of an integer selected from about 5.3 to about 5.7. In some embodiments, the EN is selected from a value greater than 5.0, 5.1, 5.2, 5.3, 5.4, 5.5, 5.6, 5.7, 5.8, and 5.9. In some embodiments, the EN is selected from a value less than 5.1, 5.2, 5.3, 5.4, 5.5, 5.6, 5.7, 5.8, 5.9, and 6.0. In some embodiments, the EN is about 5.0, 5.2, 5.4, 5.6, 5.8, or 6.0.

In some embodiments, the EN is greater than or equal to 1, such as an integer or fraction of an integer selected from about 1.0 to about 2.0. In some embodiments, the EN is a fraction of an integer selected from about 1.1 to about 1.7. In some embodiments, the EN is a fraction of an integer selected from about 1.1 to about 1.5. In some embodiments, the EN is selected from a value greater than 1.0, 1.1, 1.2, 1.3, 1.4, 1.5, 1.6, 1.7, 1.8, or 1.9. In some embodiments, the EN is selected from a value less than 1.2, 1.3, 1.4, 1.5, 1.6, 1.7, 1.8, 1.9, or 2.0. In some embodiments, the EN is about 1.0, 1.2, 1.4, 1.6, 1.8, or 2.0. In some embodiments, the EN is greater than or equal to 1, such as an integer or fraction of an integer selected from about 1.2 to about 2.2. In some embodiments, the EN is an integer or fraction of an integer selected from about 1.4 to about 2.0. In some embodiments, the EN is a fraction of an integer selected from about 1.5 to about 1.9. In some embodiments, the EN is selected from a value greater than 1.0, 1.1, 1.2, 1.3, 1.4, 1.5, 1.6, 1.7, 1.8, 1.9, 2.0, and 2.1. In some embodiments, the EN is selected from a value less than 1.2, 1.3, 1.4, 1.5, 1.6, 1.7, 1.8, 1.9, 2.0, 2.1, and 2.2. In some embodiments, the EN is about 1.0, 1.2, 1.4, 1.6, 1.8, 2.0, or 2.2.

In some embodiments, the EN is greater than or equal to 2, such as an integer or fraction of an integer selected from about 2.8 to about 3.8. In some embodiments, the EN is an integer or fraction of an integer selected from about 2.9 to about 3.5. In some embodiments, the EN is an integer or fraction of an integer selected from about 3.0 to about 3.4. In some embodiments, the EN is selected from a value greater than 2.0, 2.1, 2.2, 2.4, 2.5, 2.6, 2.7, 2.8, 2.9, 3.0, 3.1, 3.4, 3.5, 3.6, and 3.7. In some embodiments, the EN is selected from a value less than 2.2, 2.3, 2.4, 2.5, 2.6, 2.7, 2.8, 2.9, 3.0, 3.1, 3.2, 3.3, 3.4, 3.5, 3.6, 3.7, and 3.8. In some embodiments, the EN is about 2.0, 2.2, 2.4, 2.6, 2.8, 3.0, 3.2, 3.4, 3.6, or 3.8. Typically, base stocks and lubricant compositions exhibit certain lubricity, viscosity, and/or pour point characteristics. For example, in certain embodiments, suitable viscosity characteristics of the base oil may range from about 10 cSt to about 250 cSt at 40° C., and/or about 3 cSt to about 30 cSt at 100° C. In some embodiments, the compounds and compositions may exhibit viscosities within a range from about 50 cSt to about 150 cSt at 40° C., and/or about 10 cSt to about 20 cSt at 100° C.

In some embodiments, the estolide compounds and compositions may exhibit viscosities less than about 55 cSt at 40° C. or less than about 45 cSt at 40° C., and/or less than about

12 cSt at 100° C. or less than about 10 cSt at 100° C. In some embodiments, the estolide compounds and compositions may exhibit viscosities within a range from about 25 cSt to about 55 cSt at 40° C., and/or about 5 cSt to about 11 cSt at 100° C.

5 In some embodiments, the estolide compounds and compositions may exhibit viscosities within a range from about 35 cSt to about 45 cSt at 40° C., and/or about 6 cSt to about 10 cSt at 100° C. In some embodiments, the estolide compounds and compositions may exhibit viscosities within a range from about 38 cSt to about 43 cSt at 40° C., and/or about 7 cSt to about 9 cSt at 100° C.

10 In some embodiments, the estolide compounds and compositions may exhibit viscosities less than about 120 cSt at 40° C. or less than about 100 cSt at 40° C., and/or less than about 18 cSt at 100° C. or less than about 17 cSt at 100° C. In some embodiments, the estolide compounds and compositions may exhibit a viscosity within a range from about 70 cSt to about 120 cSt at 40° C., and/or about 12 cSt to about 18 cSt at 100° C. In some embodiments, the estolide compounds and compositions may exhibit viscosities within a range from about 80 cSt to about 100 cSt at 40° C., and/or about 13 cSt to about 17 cSt at 100° C. In some embodiments, the estolide compounds and compositions may exhibit viscosities within a range from about 85 cSt to about 95 cSt at 40° C., and/or about 14 cSt to about 16 cSt at 100° C.

15 In some embodiments, the estolide compounds and compositions may exhibit viscosities greater than about 180 cSt at 40° C. or greater than about 200 cSt at 40° C., and/or greater than about 20 cSt at 100° C. or greater than about 25 cSt at 100° C. In some embodiments, the estolide compounds and

20 compositions may exhibit a viscosity within a range from about 180 cSt to about 230 cSt at 40° C., and/or about 25 cSt to about 31 cSt at 100° C. In some embodiments, estolide compounds and compositions may exhibit viscosities within a range from about 200 cSt to about 250 cSt at 40° C., and/or about 25 cSt to about 35 cSt at 100° C. In some embodiments, estolide compounds and compositions may exhibit viscosities within a range from about 210 cSt to about 230 cSt at 40° C., and/or about 28 cSt to about 33 cSt at 100° C. In some embodiments, the estolide compounds and compositions may exhibit viscosities within a range from about 200 cSt to about 220 cSt at 40° C., and/or about 26 cSt to about 30 cSt at 100° C. In some embodiments, the estolide compounds and compositions may exhibit viscosities within a range from about 205 cSt to about 215 cSt at 40° C., and/or about 27 cSt to about 29 cSt at 100° C.

25 In some embodiments, the estolide compounds and compositions may exhibit viscosities less than about 45 cSt at 40° C. or less than about 38 cSt at 40° C., and/or less than about 10 cSt at 100° C. or less than about 9 cSt at 100° C. In some embodiments, the estolide compounds and compositions may exhibit a viscosity within a range from about 20 cSt to about 45 cSt at 40° C., and/or about 4 cSt to about 10 cSt at 100° C. In some embodiments, the estolide compounds and compositions may exhibit viscosities within a range from about 28 cSt to about 38 cSt at 40° C., and/or about 5 cSt to about 9 cSt at 100° C. In some embodiments, the estolide compounds and compositions may exhibit viscosities within a range from about 30 cSt to about 35 cSt at 40° C., and/or about 6 cSt to about 8 cSt at 100° C.

30 In some embodiments, the estolide compounds and compositions may exhibit viscosities less than about 80 cSt at 40° C. or less than about 70 cSt at 40° C., and/or less than about 14 cSt at 100° C. or less than about 13 cSt at 100° C. In some embodiments, the estolide compounds and compositions may exhibit a viscosity within a range from about 50 cSt to about 80 cSt at 40° C., and/or about 8 cSt to about 14 cSt at 100° C.

35 In some embodiments, the estolide compounds and compositions may exhibit viscosities within a range from about 60 cSt to about 70 cSt at 40° C., and/or about 9 cSt to about 13 cSt

at 100° C. In some embodiments, the estolide compounds and compositions may exhibit viscosities within a range from about 63 cSt to about 68 cSt at 40° C., and/or about 10 cSt to about 12 cSt at 100° C.

In some embodiments, the estolide compounds and compositions may exhibit viscosities greater than about 120 cSt at 40° C. or greater than about 130 cSt at 40° C., and/or greater than about 15 cSt at 100° C. or greater than about 18 cSt at 100° C. In some embodiments, the estolide compounds and compositions may exhibit a viscosity within a range from about 120 cSt to about 150 cSt at 40° C., and/or about 16 cSt to about 24 cSt at 100° C. In some embodiments, the estolide compounds and compositions may exhibit viscosities within a range from about 130 cSt to about 160 cSt at 40° C., and/or about 17 cSt to about 28 cSt at 100° C. In some embodiments, the estolide compounds and compositions may exhibit viscosities within a range from about 130 cSt to about 145 cSt at 40° C., and/or about 17 cSt to about 23 cSt at 100° C. In some embodiments, the estolide compounds and compositions may exhibit viscosities within a range from about 135 cSt to about 140 cSt at 40° C., and/or about 19 cSt to about 21 cSt at 100° C. In some embodiments, the estolide compounds and compositions may exhibit viscosities of about 1, 2, 3, 4, 5, 6, 7, 8, 9, 10, 11, 12, 13, 14, 15, 16, 17, 18, 19, 20, 21, 22, 23, 24, 25, 26, 27, 28, 29, 30, 32, 34, 36, 38, 40, 42, 44, 46, 48, 50, 55, 60, 65, 70, 75, 80, 85, 90, 95, 100, 110, 120, 130, 140, 150, 160, 170, 180, 190, 200, 210, 220, 230, 240, 250, 260, 270, 280, 290, 300, 350, or 400 cSt at 40° C. In some embodiments, the estolide compounds and compositions may exhibit viscosities of about 1, 2, 3, 4, 5, 6, 7, 8, 9, 10, 11, 12, 13, 14, 15, 16, 17, 18, 19, 20, 21, 22, 23, 24, 25, 26, 27, 28, 29, and 30 cSt at 100° C. In certain embodiments, estolides may exhibit desirable low-temperature pour point properties. In some embodiments, the estolide compounds and compositions may exhibit a pour point lower than about -25° C., about -35° C., -40° C., or even about -50° C. In some embodiments, the estolide compounds and compositions have a pour point of about -25° C. to about -45° C. In some embodiments, the pour point falls within a range of about -30° C. to about -40° C., about -34° C. to about -38° C., about -30° C. to about -45° C., -35° C. to about -45° C., 34° C. to about -42° C., about -38° C. to about -42° C., or about 36° C. to about -40° C. In some embodiments, the pour point falls within the range of about -27° C. to about -37° C., or about -30° C. to about -34° C. In some embodiments, the pour point falls within the range of about -25° C. to about -35° C., or about -28° C. to about -32° C. In some embodiments, the pour point falls within the range of about -28° C. to about -38° C., or about -31° C. to about -35° C. In some embodiments, the pour point falls within the range of about -31° C. to about -41° C., or about -34° C. to about -38° C. In some embodiments, the pour point falls within the range of about -40° C. to about -50° C., or about -42° C. to about -48° C. In some embodiments, the pour point falls within the range of about -50° C. to about -60° C., or about -52° C. to about -58° C. In some embodiments, the upper bound of the pour point is less than about -35° C., about -36° C., about -37° C., about -38° C., about -39° C., about -40° C., about -41° C., about -42° C., about -43° C., about -44° C., or about -45° C. In some embodiments, the lower bound of the pour point is greater than about -70° C., about -69° C., about -68° C., about -67° C., about -66° C., about -65° C., about -64° C., about -63° C., about -62° C., about -61° C., about -60° C., about -59° C., about -58° C., about -57° C., about -56° C., -55° C., about -54° C., about -53° C., about -52° C., -51, about -50° C., about -49° C., about -48° C., about -47° C., about -46° C., or about -45° C.

In addition, in certain embodiments, the estolides may exhibit decreased Iodine Values (IV) when compared to estolides prepared by other methods. IV is a measure of the

degree of total unsaturation of an oil, and is determined by measuring the amount of iodine per gram of estolide (cg/g). In certain instances, oils having a higher degree of unsaturation may be more susceptible to creating corrosiveness and deposits, and may exhibit lower levels of oxidative stability. Compounds having a higher degree of unsaturation will have more points of unsaturation for iodine to react with, resulting in a higher IV. Thus, in certain embodiments, it may be desirable to reduce the IV of estolides in an effort to increase the oil's oxidative stability, while also decreasing harmful deposits and the corrosiveness of the oil.

In some embodiments, estolide compounds and compositions described herein have an IV of less than about 40 cg/g or less than about 35 cg/g. In some embodiments, estolides have an IV of less than about 30 cg/g, less than about 25 cg/g, less than about 20 cg/g, less than about 15 cg/g, less than about 10 cg/g, or less than about 5 cg/g. The IV of a composition may be reduced by decreasing the estolide's degree of unsaturation. This may be accomplished by, for example, by increasing the amount of saturated capping materials relative to unsaturated capping materials when synthesizing the estolides. Alternatively, in certain embodiments, IV may be reduced by hydrogenating estolides having unsaturated caps.

The present disclosure further relates to methods of making estolides according to Formulas I and II. By way of example, the reaction of one or more unsaturated fatty acids with one or more dicarboxylic acids, and the esterification of the resulting free acid estolide, are illustrated and discussed in the following Schemes 1-3. The particular structural formulas used to illustrate the reactions correspond to those for synthesis of compounds according to Formula I; however, the methods apply equally to the synthesis of compounds according to Formula II, with use of compounds having structure corresponding to R<sub>3</sub> and R<sub>4</sub> with reactive sites of unsaturation.

As discussed in the schemes outlined further below, compound 102 represents an unsaturated fatty acid that may serve as the basis for preparing the dicarboxylate-capped estolide compounds described herein.

Scheme 1



In Scheme 1, wherein x is, independently for each occurrence, an integer selected from 0 to 20, y is, independently for each occurrence, an integer selected from 0 to 20, n is an integer greater than or equal to 0, W is  $-\text{CH}_2-$  or

$-\text{CH}=\text{CH}-$ , and  $z$  is an integer selected from 1 to 40, unsaturated fatty acid 102 may be added to a solution containing an equal or excess amount of dicarboxylic acid 100 and a catalyst to form dicarboxylate-capped free acid estolide 104. Depending on the desired product, the slow addition of unsaturated fatty acid 102 to a solution of dicarboxylic acid 100 and catalyst may help to maximize the addition of dicarboxylic acid 100 to a single unsaturated fatty acid 102, while minimizing the formation of larger oligomers (e.g., where  $n > 0$ ) and/or the addition of a second molecule of unsaturated fatty acid 102 to the unreacted (free) carboxylic acid residue of dicarboxylic acid 100. Any suitable catalyst may be implemented to catalyze the formation of free acid estolide 104, including but not limited to Lewis acids, homogenous acids and/or strong acids or other proton sources such as hydrochloric acid, sulfuric acid, perchloric acid, nitric acid, triflic acid, and the like. In certain embodiments, unsaturated fatty acid 102 may be replaced with a hydroxy fatty acid (e.g., 12-hydroxystearic acid), wherein free acid estolide 104 is formed via a condensation reaction between the free hydroxyl residue of said hydroxy fatty acid and a carboxylic acid residue of dicarboxylic acid 100.

the like. In certain embodiments, unsaturated fatty acid 102 may be replaced with a hydroxy fatty acid (e.g., 12-hydroxystearic acid), wherein free acid diestolide 200 is formed via a condensation reaction between the free hydroxyl residues of two hydroxy fatty acid molecules and the two carboxylic acid residues of dicarboxylic acid 100.

Scheme 3



Scheme 2



Alternatively, in Scheme 2, wherein  $x$  and  $x'$  are, independently for each occurrence, an integer selected from 0 to 20,  $y$  and  $y'$  are, independently for each occurrence, an integer selected from 0 to 20,  $n$  and  $n'$  are, independently for each occurrence, an integer greater than or equal to 0,  $W$  is  $-\text{CH}_2-$  or  $-\text{CH}=\text{CH}-$ , and  $z$  is an integer selected from 1 to 40, dicarboxylic acid 100 and a catalyst may be added to unsaturated fatty acid 102 to form free acid diestolide 200. In certain embodiments, it may be desirable to start the synthesis with a solution of at least two equivalents of unsaturated fatty acid 100, and the catalyst, followed by the slow addition of one equivalent of dicarboxylic acid 100, which may help to increase oligomerization and/or the addition of a molecule of unsaturated acid 102 to each of the carboxylic acid residues of dicarboxylic acid 100. Any suitable catalyst may be implemented to catalyze the formation of free acid diestolide 200, including but not limited to Lewis acids, homogenous acids and/or strong acids or proton sources such as hydrochloric acid, sulfuric acid, perchloric acid, nitric acid, triflic acid, and

50

55

60

65



In Scheme 3, wherein  $W$ ,  $z$ ,  $x$ ,  $y$ , and  $n$  are as defined above, free acid estolide 104 may be esterified by any suitable procedure known to those of skilled in the art, such as acid-catalyzed reduction with alcohol 302, to yield esterified dicar-

23

boxylate-capped estolide 304, wherein  $R_2$  represents an optionally substituted alkyl group that is saturated or unsaturated, and branched or unbranched. This synthetic route may also be suitable for the esterification of free acid diestolide estolide 200. Other exemplary methods may include other types of Fischer esterification, such as those using Lewis acid catalysts such as  $BF_3$ .

24

ids, and the like. Other suitable uses may include marine applications, where biodegradability and toxicity are of concern. In certain embodiments, the nontoxic nature of the estolides described herein may also make them suitable for use as lubricants in the cosmetic and food industries. In certain embodiments, the estolides described herein may be suitable for use as pour-point depressants.

Scheme 4



In Scheme 4, wherein  $z$ ,  $x$ ,  $y$ , and  $n$  are as defined above, unsaturated fatty acid 400 may undergo oligomerization under catalytic conditions (e.g., Bronsted or Lewis acid catalyst) to provide unsaturated free-acid estolide 402. Exposure of unsaturated free-acid estolide 402 to oxidative conditions may result in the cleavage of the capping chain residue double bond, resulting in the formation of dicarboxylate-capped estolide 404. Exemplary oxidative conditions may include, but are not limited to, ozonolysis and acidic  $KMnO_4$ . Alternatively, unsaturated free-acid estolide 402 may undergo metathesis with an unsaturated fatty acid reactant to provide dicarboxylate-capped estolide 406. Exemplary metathesis conditions include the use of a metathesis catalyst (e.g., Grubbs' catalyst) with an unsaturated free fatty acid or unsaturated fatty ester, wherein  $R_2$  represents hydrogen or an optionally substituted alkyl group that is saturated or unsaturated, and branched or unbranched. If desired, the unsaturated dicarboxylate cap of estolide 406 may be hydrogenated using any suitable methods known to those of skill in the art.

As discussed above, in certain embodiments, the estolides described herein may have improved properties which render them useful as base stocks or additives for biodegradable lubricant applications. Such applications may include, without limitation, crankcase oils, gearbox oils, hydraulic fluids, drilling fluids, two-cycle engine oils, greases, dielectric flu-

In certain embodiments, estolide compounds may meet or exceed one or more of the specifications for certain end-use applications, without the need for conventional additives. For example, in certain instances, high-viscosity lubricants, such as those exhibiting a kinematic viscosity of greater than about 120 cSt at 40° C., or even greater than about 200 cSt at 40° C., may be desirable for particular applications such as gearbox or wind turbine lubricants. Prior-known lubricants with such properties typically also demonstrate an increase in pour point as viscosity increases, such that prior lubricants may not be suitable for such applications in colder environments. However, in certain embodiments, the counterintuitive properties of certain compounds described herein (e.g., increased EN provides estolides with higher viscosities while retaining, or even decreasing, the oil's pour point) may make higher-viscosity estolides particularly suitable for such specialized applications.

Similarly, the use of prior-known lubricants in colder environments may generally result in an unwanted increase in a lubricant's viscosity. Thus, depending on the application, it may be desirable to use lower-viscosity oils at lower temperatures. In certain circumstances, low-viscosity oils may include those exhibiting a viscosity of lower than about 50 cSt at 40° C., or even about 40 cSt at 40° C. Accordingly, in certain embodiments, the low-viscosity estolides described herein may provide end users with a suitable alternative to high-viscosity lubricants for operation at lower temperatures.

In some embodiments, it may be desirable to prepare lubricant compositions comprising one or more of the estolide compounds described herein. For example, in certain embodiments, the estolides described herein may be blended with one or more additives selected from polyalphaolefins, synthetic esters, polyalkylene glycols, mineral oils (Groups I, II, and III), pour point depressants, viscosity modifiers, anti-corrosives, antiwear agents, detergents, dispersants, colorants, antifoaming agents, and demulsifiers. In addition, or in the alternative, in certain embodiments, the estolides described herein may be co-blended with one or more synthetic or petroleum-based oils to achieve the desired viscosity and/or pour point profiles. In certain embodiments, the estolides described herein also mix well with gasoline, so that they may be useful as fuel components or additives.

In all of the foregoing examples, the compounds described may be useful alone, as mixtures, or in combination with other compounds, compositions, and/or materials.

Methods for obtaining the novel compounds described herein will be apparent to those of ordinary skill in the art, suitable procedures being described, for example, in the examples below, and in the references cited herein.

## EXAMPLES

### Analytics

Nuclear Magnetic Resonance: NMR spectra were collected using a Bruker Avance 500 spectrometer with an absolute frequency of 500.113 MHz at 300 K using  $\text{CDCl}_3$  as the solvent. Chemical shifts were reported as parts per million from tetramethylsilane. The formation of a secondary ester link between fatty acids, indicating the formation of estolide, was verified with  $^1\text{H}$  NMR by a peak at about 4.84 ppm.

Estolide Number (EN): The EN was measured by GC analysis. It should be understood that the EN of a composition specifically refers to EN characteristics of any estolide compounds present in the composition. Accordingly, an estolide composition having a particular EN may also comprise other components, such as natural or synthetic additives, other non-estolide base oils, fatty acid esters, e.g., triglycerides, and/or fatty acids, but the EN as used herein, unless otherwise indicated, refers to the value for the estolide fraction of the estolide composition.

Iodine Value (IV): The iodine value is a measure of the degree of total unsaturation of an oil. IV is expressed in terms of centigrams of iodine absorbed per gram of oil sample. Therefore, the higher the iodine value of an oil the higher the level of unsaturation is of that oil. The IV may be measured and/or estimated by GC analysis. Where a composition includes unsaturated compounds other than estolides as set forth in Formula I and II, the estolides can be separated from other unsaturated compounds present in the composition prior to measuring the iodine value of the constituent estolides. For example, if a composition includes unsaturated fatty acids or triglycerides comprising unsaturated fatty acids, these can be separated from the estolides present in the composition prior to measuring the iodine value for the one or more estolides.

Acid Value: The acid value is a measure of the total acid present in an oil. Acid value may be determined by any suitable titration method known to those of ordinary skill in the art. For example, acid value may be determined by the amount of KOH that is required to neutralize a given sample of oil, and thus may be expressed in terms of mg KOH/g of oil.

Gas Chromatography (GC): GC analysis was performed to evaluate the estolide number (EN) and iodine value (IV) of the estolides. This analysis was performed using an Agilent

6890N series gas chromatograph equipped with a flame-ionization detector and an autosampler/injector along with an SP-2380 30 m $\times$ 0.25 mm i.d. column.

The parameters of the analysis were as follows: column flow at 1.0 mL/min with a helium head pressure of 14.99 psi; split ratio of 50:1; programmed ramp of 120-135° C. at 20° C./min, 135-265° C. at 7° C./min, hold for 5 min at 265° C.; injector and detector temperatures set at 250° C.

Measuring EN and IV by GC: To perform these analyses, the fatty acid components of an estolide sample were reacted with MeOH to form fatty acid methyl esters by a method that left behind a hydroxy group at sites where estolide links were once present. Standards of fatty acid methyl esters were first analyzed to establish elution times.

Sample Preparation: To prepare the samples, 10 mg of estolide was combined with 0.5 mL of 0.5M KOH/MeOH in a vial and heated at 100° C. for 1 hour. This was followed by the addition of 1.5 mL of 1.0 M  $\text{H}_2\text{SO}_4$ /MeOH and heated at 100° C. for 15 minutes and then allowed to cool to room temperature. One (1) mL of  $\text{H}_2\text{O}$  and 1 mL of hexane were then added to the vial and the resulting liquid phases were mixed thoroughly. The layers were then allowed to phase separate for 1 minute. The bottom  $\text{H}_2\text{O}$  layer was removed and discarded. A small amount of drying agent ( $\text{Na}_2\text{SO}_4$  anhydrous) was then added to the organic layer after which the organic layer was then transferred to a 2 mL crimp cap vial and analyzed.

EN Calculation: The EN is measured as the percent hydroxy fatty acids divided by the percent non-hydroxy fatty acids. As an example, a dimer estolide would result in half of the fatty acids containing a hydroxy functional group, with the other half lacking a hydroxy functional group. Therefore, the EN would be 50% hydroxy fatty acids divided by 50% non-hydroxy fatty acids, resulting in an EN value of 1 that corresponds to the single estolide link between the capping fatty acid and base fatty acid of the dimer.

IV Calculation: The iodine value is estimated by the following equation based on ASTM Method D97 (ASTM International, Conshohocken, Pa.):

$$IV = \sum 100 \times \frac{A_f \times MW_1 \times db}{MW_f}$$

$A_f$ =fraction of fatty compound in the sample

$MW_f$ =253.81, atomic weight of two iodine atoms added a double bond

$db$ =number of double bonds on the fatty compound

$MW_f$ =molecular weight of the fatty compound

Other Measurements: Except as otherwise described, pour point is measured by ASTM Method D97-96a, cloud point is measured by ASTM Method D2500, viscosity/kinematic viscosity is measured by ASTM Method D445-97, viscosity index is measured by ASTM Method D2270-93 (Reapproved 1998), specific gravity is measured by ASTM Method D4052, flash point is measured by ASTM Method D92, evaporative loss is measured by ASTM Method D5800, vapor pressure is measured by ASTM Method D5191, and acute aqueous toxicity is measured by Organization of Economic Cooperation and Development (OECD) 203.

### Example 1

The acid catalyst reaction was conducted in a 50 gallon Pfaudler RT-Series glass-lined reactor. Oleic acid (65 Kg, OL 700, Twin Rivers) was added to the reactor with 70% perchloro-

27

ric acid (992.3 mL, Aldrich Cat#244252) and heated to 60° C. in vacuo (10 torr abs) for 24 hrs while continuously being agitated. After 24 hours the vacuum was released. 2-Ethylhexanol (29.97 Kg) was then added to the reactor and the vacuum was restored. The reaction was allowed to continue under the same conditions (60° C., 10 torr abs) for 4 more hours. At which time, KOH (645.58 g) was dissolved in 90% ethanol/water (5000 mL, 90% EtOH by volume) and added to the reactor to quench the acid. The solution was then allowed to cool for approximately 30 minutes. The contents of the reactor were then pumped through a 1 micron ( $\mu$ ) filter into an accumulator to filter out the salts. Water was then added to the accumulator to wash the oil. The two liquid phases were thoroughly mixed together for approximately 1 hour. The solution was then allowed to phase separate for approximately 30 minutes. The water layer was drained and disposed of. The organic layer was again pumped through a 1 $\mu$  filter back into the reactor. The reactor was heated to 60° C. in vacuo (10 torr abs) until all ethanol and water ceased to distill from solution. The reactor was then heated to 100° C. in vacuo (10 torr abs) and that temperature was maintained until the 2-ethylhexanol ceased to distill from solution. The remaining material was then distilled using a Myers 15 Centrifugal Distillation still at 200° C. under an absolute pressure of approximately 12 microns (0.012 ton) to remove all monoester material, leaving behind estolides.

#### Example 2

Estolides are prepared according to the method set forth in Example 1, except the oleic acid starting material is replaced with an equal weight of a combination of 1,10-Decanedicarboxylic acid (1.2 equiv., Cathay Indus.) and Oleic acid (1 equiv., OL 700, Twin Rivers), and the volume of 2-ethylhexanol is doubled. Purification and distillation to remove unreacted starting materials provides a mixture of estolide products, including esterified dicarboxylate-capped estolides and esterified diestolides.

#### Example 3

The acid catalyst reaction is conducted in a 3-neck flask equipped with stir bar, thermometer, and distillation column. 1,10-Decanedicarboxylic acid (12 equiv., Cathay Indus.) is added to the flask with 70% perchloric acid (1.0 equiv., Aldrich Cat#244252) and heated to 60° C. in vacuo (10 torr abs) while continuously being agitated. Oleic acid (10 equiv., OL 700, Twin Rivers) is added dropwise by syringe pump over a period of about 12-18 hours. Heating the vessel under reduced pressure is continued for a total of about 24 hours, after which the vacuum is released. At which time, the acid catalyst is quenched with a molar equivalent of KOH dissolved in 90% ethanol in water for 30 min under continuous agitation. The solution is then allowed to cool for approximately 30 minutes. The contents of the flask are then pumped through a 1 micron ( $\mu$ ) filter into an accumulator to filter out the salts. Water is then added to the accumulator to wash the oil. The two liquid phases are thoroughly mixed together for approximately 1 hour. The solution is then allowed to phase separate for approximately 30 minutes. The water layer is drained and disposed of. The organic layer is again pumped through a 1 $\mu$  filter back into the flask. The reactor is heated to 60° C. in vacuo (10 torr abs) until all ethanol and water ceased to distill from solution. Dicarboxylate-capped estolides are then separated from unreacted dicarboxylic and fatty acids

28

using any suitable methods known to those of skill in the art, such as distillation or chromatography.

#### Example 4

5 The acid catalyst reaction is conducted in a 3-neck flask equipped with stir bar, thermometer, and distillation column. Oleic acid (12 equiv., OL 700, Twin Rivers) is added to the flask with 70% perchloric acid (1.0 equiv., Aldrich Cat#244252) and heated to 60° C. in vacuo (10 torr abs) while continuously being agitated. 1,10-Decanedicarboxylic acid (10 equiv., Cathay Indus.) is added dropwise by syringe pump over a period of about 12-18 hours. Heating the vessel under reduced pressure is continued for a total of about 24 hours, 10 after which the vacuum is released. At which time, the acid catalyst is quenched with a molar equivalent of KOH dissolved in 90% ethanol in water for 30 min under continuous agitation. The solution is then allowed to cool for approximately 30 minutes. The contents of the flask are then pumped 15 through a 1 micron ( $\mu$ ) filter into an accumulator to filter out the salts. Water is then added to the accumulator to wash the oil. The two liquid phases are thoroughly mixed together for approximately 1 hour. The solution is then allowed to phase 20 separate for approximately 30 minutes. The water layer is drained and disposed of. The organic layer is again pumped through a 1 $\mu$  filter back into the flask. The reactor is heated to 60° C. in vacuo (10 torr abs) until all ethanol and water ceased to distill from solution. Diestolides are then separated from 25 unreacted dicarboxylic and fatty acids using any suitable methods known to those of skill in the art, such as distillation or chromatography.

#### Example 5

35 Separately, the dicarboxylate-capped estolide and diestolide products of Examples 3 and 4, respectively, are placed in a round bottom flask equipped with a stir bar and a solution of  $\text{BF}_3 \cdot \text{OEt}_2$  (0.15 equiv.) and 2-EH (2.2 equiv.) The solutions are then heated to 60° C. under stirring for 3-4 hours. The 40 reaction mixtures are then cooled to room temperature and quenched with water. The oils are separated and washed with brine, followed by drying over sodium sulfate. The esterified products are recovered from any unreacted 2-EH using any suitable methods known to those of skill in the art, such as distillation or chromatography.

45 The invention claimed is:

1. At least one compound of Formula I:

Formula I



wherein

x is, independently for each occurrence, an integer selected

from 2 to 8;

y is, independently for each occurrence, an integer selected from 0 to 20;

29

- z is an integer selected from 4 to 18;  
 n is an integer selected from 0 to 6;  
 W is, independently for each occurrence, selected from  
 $-\text{CH}_2-$  and  $-\text{CH}=\text{CH}-$ ;  
 R<sub>5</sub> is selected from hydrogen, unsubstituted alkyl that is 5  
 saturated or unsaturated, and branched or unbranched,  
 and an estolide residue; and  
 R<sub>2</sub> is selected from hydrogen and unsubstituted alkyl that is  
 saturated or unsaturated, and branched or unbranched,  
 wherein each fatty acid chain residue of said at least one  
 compound is unsubstituted.  
 2. The at least one compound according to claim 1, wherein  
 x+y is, independently for each occurrence, an integer selected  
 from 13 to 15.  
 3. The at least one compound according to claim 1, wherein  
 z is an integer selected from 6 to 16.  
 4. The at least one compound according to claim 1, wherein  
 z is 10.  
 5. The at least one compound according to claim 1, wherein  
 n is 0.  
 6. The at least one compound according to claim 1, wherein  
 R<sub>5</sub> and R<sub>2</sub> are hydrogen.  
 7. The at least one compound according to claim 1, wherein  
 R<sub>2</sub> is a branched or unbranched C<sub>1</sub> to C<sub>20</sub> alkyl that is sat-  
 rated or unsaturated.  
 8. The at least one compound according to claim 1, wherein  
 R<sub>5</sub> is a branched or unbranched C<sub>1</sub> to C<sub>20</sub> alkyl that is sat-  
 rated or unsaturated.  
 9. The at least one compound according to claim 1, wherein  
 R<sub>5</sub> is an estolide residue selected from the structure of For-  
 mula III:



30

- wherein  
 x', independently for each occurrence, is an integer  
 selected from 0 to 20;  
 y', independently for each occurrence, is an integer  
 selected from 0 to 20;  
 n' is an integer selected from 0 to 6; and  
 R<sub>6</sub> is selected from hydrogen and unsubstituted alkyl  
 that is saturated or unsaturated, and branched or  
 unbranched.  
 10. The at least one compound according to claim 9,  
 wherein  
 x' is, independently for each occurrence, an integer  
 selected from 7 and 8; and  
 y' is, independently for each occurrence, an integer  
 selected from 7 and 8.  
 11. The at least one compound according to claim 9,  
 wherein n' is 0.  
 12. The at least one compound according to claim 1,  
 wherein  
 n is 0;  
 x is, independently for each occurrence, an integer selected  
 from 7 and 8;  
 y is, independently for each occurrence, an integer selected  
 from 7 and 8; and  
 R<sub>5</sub> and R<sub>2</sub> are independently selected from branched C<sub>4</sub> to  
 C<sub>20</sub> alkyl.  
 13. The at least one compound according to any claim 3,  
 wherein z is 16.  
 14. The at least one compound according to claim 1,  
 wherein W is  $-\text{CH}_2-$ .  
 15. The at least one compound according to claim 1,  
 wherein y is 0 for each occurrence.  
 16. The at least one compound according to claim 15,  
 wherein x is, independently for each occurrence, and integer  
 selected from 7 and 8.  
 17. The at least one compound according to claim 16, R<sub>5</sub>  
 and R<sub>2</sub> are independently selected from unsubstituted C<sub>1</sub> to  
 C<sub>20</sub> alkyl that is saturated and branched or unbranched.  
 18. The at least one compound according to claim 16,  
 wherein R<sub>5</sub> and R<sub>2</sub> are independently selected from branched  
 C<sub>4</sub> to C<sub>20</sub> alkyl.  
 19. The at least one compound according to claim 18,  
 wherein R<sub>5</sub> and R<sub>2</sub> are 2-ethylhexyl.  
 20. The at least one compound according to claim 9,  
 wherein z is an integer selected from 6 to 16.

\* \* \* \* \*